

# United States Patent Office

2,860,040

Patented Nov. 11, 1958

1

2,860,040

## PETROLEUM DISTILLATE FUELS

Fred B. Fischl, Springfield, and George A. Weisgerber, Iselin, N. J., assignors to Esso Research and Engineering Company, a corporation of Delaware

No Drawing. Application May 25, 1955  
Serial No. 511,102

9 Claims. (Cl. 44—72)

This invention pertains to improved distillate petroleum fuel oil compositions and to a method of preparing the same. The invention relates to both straight run and cracked type petroleum fuels, but it particularly concerns those petroleum fuels that contain at least 10% by volume petroleum fractions that are derived from catalytic or thermal cracking operations. The invention especially concerns petroleum distillate fuels that are derived at least in part from cracking operations, that are stabilized against sediment formations, and that possess the ability to inhibit the corrosion of ferruginous metals which are in contact with water. The invention is especially adapted for the stabilization of cracked fuel oils which are maintained in storage for extended periods of time; and the invention is further particularly adapted for the prevention and reduction of corrosion in fuel storage tanks, petroleum pipe lines, oil cargo vessels, etc.

Petroleum distillate fuels as such are well known in the art and include heating oils, kerosenes, diesel fuels, industrial fuel oils and the like. These fuels constitute major products in the petroleum refining industry; and, accordingly, considerable effort has been expended by this industry in an effort to maintain and improve the quality of these products. In years past, these fuels consisted primarily of straight-run stocks, but in more recent years it has been necessary to include substantial amounts of cracked stocks within the fuel. With the inclusion of these cracked stocks, the refiners have encountered several problems—a primary problem being one of better stabilization of the fuels against the formation of sediment during extended storage periods. The precise reasons and the mechanism for the formation of the sediment are not known to any degree of certainty, but it is recognized that the presence of the cracked materials is in some way largely responsible for the sediment.

In an effort to overcome the sediment formation problem, petroleum refiners have resorted to a number of tactics including the utilization of new refining techniques as well as the use of various additives. These additives have included metal naphthenates, metal sulfonates, salts of alkyl phenol sulfides, various amine compounds and the like. These materials have been successful to a degree in overcoming the sedimentation problem, but a continuing search is still in progress for still better additives to serve this function. In this connection it has recently been observed that some of the sediment-stabilizing agents are effective in varying degrees in preventing the formation of sediment in fuel oils depending apparently upon the amount and origin of the cracked constituents in the oils. Of particular interest is the observation that, when these agents are employed in more extensively cracked stocks or in fuel oils that contain large amounts of cracked stocks, the degree of sedimentation is often actually greater than would be expected even without the sediment-stabilizing agents. The reason for this anomalous condition is not known as yet, but it appears that an ineffective amount of stabilizing agent fails to prevent the

2

sediment from forming; and when the sediment does form, it tends to precipitate the agent along with it. Thus, it is extremely desirable to find and develop sediment-stabilizing agents which are more effective in inhibiting sediment formation than are the materials that are presently employed for this purpose.

In addition to the sediment forming problem, a rather serious corrosion problem exists in storage tanks, oil cargo vessels, pipe lines, etc. which are employed for the storage and/or transportation of distillate fuel oils. It will be appreciated and it is a well known fact in the art that these storage vessels and transportation media generally contain small amounts of water in addition to the distillate fuel oils, and it has been observed that the presence of the water (along or in conjunction with the fuel oils) gives rise to a peculiar form of corrosive action. The type of corrosion is perhaps best designated as a "pitting" action in that the metallic surfaces affected are penetrated by relatively small diameter, but deep pits. When these pits are deep, enough to penetrate entirely through the metal container or vessel, leakage or failure of the vessel or container may occur. In any event, extensive fuel losses may occur and repair of the vessels or pipe lines must be made. All of these results are expensive, and it is eminently desirable to avoid their occurrence.

It is an object of the present invention to overcome and avoid the sediment formation and corrosion problems that are associated with the manufacture and handling of petroleum distillate fuels. It is especially an object of the invention to provide distillate fuel oils that contain in excess of 10 vol. percent cracked stocks with minor proportions of a complex additive agent which is capable of simultaneously preventing both of the aforementioned problems, i. e. corrosion and sediment formation.

In accordance with the present invention, a petroleum distillate fuel oil and particularly one containing at least 10 vol. percent cracked stocks is stabilized against sediment formation and is also simultaneously endowed with corrosion inhibiting qualities by the incorporation therein of a minor but effective amount of a complex reaction product formed by reacting a particular type of sulfonate compound with particular inorganic salts. The precise sulfonates and inorganic salts that may be employed for this purpose will be described in detail later in this description.

As mentioned earlier, the fuel oil components of the present fuel oil compositions are petroleum distillate fractions such as are commonly designated as kerosenes, diesel fuels, distillate heating oils, distillate industrial fuel oils, etc. The invention has application to those petroleum distillate fuel oils that boil within the range from about 325° F. to 675° F. and that possess specific gravities of about 23 to 40° API. Typical inspections of such petroleum distillates are as follows:

|                           |            |
|---------------------------|------------|
| Gravity, ° API            | 23 to 40   |
| Initial b. pt., ° F       | 325 to 360 |
| Final b. pt., ° F         | 550 to 675 |
| Sulfur, wt. percent       | 0.1 to 1.5 |
| Color, Robinson           | 10 to 25+  |
| Viscosity, SUS, at 100° F | 30 to 60   |
| Flash point, ° F          | 115 to 160 |

As stated above, fuel oils that are particularly benefitted by this invention are characterized by possessing at least about 10 vol. percent constituents that are derived from cracking operations. The fuel oils may be entirely composed of cracked stocks, but the invention is especially directed toward the stabilization of those fuel oils that contain about 20 to 80 vol. percent of such stocks.

It will be appreciated that the cracked components of the present fuel oil compositions may be derived in part

or entirely from thermal and/or catalytic type cracking operations. Thus, typical fuel oils that may be employed in accordance with the invention are fuel oils that contain from 20 to 90 vol. percent straight run components, 0 to 80 vol. percent thermally cracked components, and 0 to 80 vol. percent catalytically cracked components. It will be noted that stocks derived from other operations such as reforming, hydroforming, hydrofining, coking, steam cracking and the like may also be utilized.

The inorganic salts that are used in the practice of the present invention include the salts of nitrous acid, wherein the cationic or metal portions of the salts are selected from the group consisting of the ammonium radical and the metals of group 1 of the periodic table. Thus, cations that are suitable include the ammonium radical, sodium, potassium and lithium. Of these cations, the ammonium radical and sodium are preferred and the latter cation is particularly preferred. It will be appreciated, of course, that these various salts may be used either singly or in unison with one another.

The sulfonates that are utilized in the compositions of the present invention are the salts of alkyl monocyclic and bicyclic aryl sulfonic acids wherein the cationic portion of the sulfonates is preferably the ammonium radical. Metals selected from group 1 or group 2 of the periodic table such as sodium, potassium, lithium, calcium and barium may also be employed, but the ammonium radical possesses unique advantages, partially because of its ashless nature. Once again, these salts may be used either separately, or in combination with one another.

Sulfonic acids that may be utilized in the practice of the present invention include the oil-soluble petroleum sulfonic acids that are derived from sulfonating petroleum distillate fractions with sulfuric acid, sulfuric trioxide, and the like. Acids of this type that are particularly effective for the purposes of this invention include those that possess molecular weights within the range from about 300 to 650 and especially about 450 to 550. Acids of this character and their manner of preparation are well known in the art and a detailed discussion of these features is therefore not considered to be necessary in the present description.

A preferred class of sulfonic acids for use in preparing the above sulfonate salts consists of the mono-sulfonated alkylated mono- and/or bi-cyclic aromatic sulfonic acids which are formed by alkylating an aromatic nucleus with an alkyl radical and thereafter sulfonating the alkylated product with sulfuric acid. The resulting sulfonic acid is then conveniently neutralized with ammonia or an alkali, or one of the aforementioned desired metals to form the corresponding ammonium or metal sulfonate salt. Any excess or unreacted alkali, water, etc. may be separated from the product by decantation, filtration, or the like. In general, it is preferred that the aromatic nucleus of the sulfonate salts be a simple benzene ring.

The alkyl group or groups of the alkylated mono- and bi-cyclic aromatic compounds may contain a total number of carbon atoms up to about 40, and the group or groups may be straight chain and/or branched in structure. Preferred sulfonic acids for use in the invention are ones that are derived from the sulfonation of mono-, di-, and tri-alkyl substituted benzene or naphthalene. Compounds that are especially preferred for sulfonation to the corresponding sulfonic acids are those having the structure



wherein R<sub>1</sub> is a hydrogen atom or an alkyl group that contains from 6-12 carbon atoms, and R<sub>2</sub> is an alkyl

group containing from about 12-24 carbon atoms. It will be noted that an alkylated naphthalene may be substituted for the alkylated benzene shown in the above structure.

5 It is further preferred that the cumulative number of carbon atoms among the alkyl groups of the alkylated mono- and bi-cyclic compounds illustrated above be about 12-36 and preferably about 24. Thus, specific examples of alkylated aromatic compounds of this type 10 include didodecyl benzene, tridodecyl benzene, octadecyl benzene, tetracosyl benzene, hexyl dodecyl benzene, hexyl octadecyl benzene, etc. An especially preferred alkylated monocyclic aryl sulfonic acid is the sulfonic acid of didodecyl benzene.

Especially preferred alkyl mono aryl sulfonic acids are the acids that are formed by alkylating benzene with an olefin polymer such as polypropylene or polybutene or with copolymers of propylene and butylenes, and thereafter sulfonating the resulting alkylate. The class 15 of compounds may thus be identified as the polypropyl or polybutyl benzene sulfonic acids. Compounds of this type are well-known in the art as well as the methods for their manufacture. Insofar as the present invention is concerned, the compounds of this type that are of especial interest are the compounds wherein the alkyl groups are derived from olefin polymers and contain from 9-18 carbon atoms each and especially about 12 carbon atoms, the total number of alkyl carbon atoms in any given benzene sulfonic acid being 40 or less, 20 preferably 12-36, and especially about 24. An especially preferred compound of this type for use in the present invention is the ammonium salt of didodecyl benzene sulfonic acid wherein the alkyl radicals are tetrapropylene. The ammonium sulfonate may be used 25 in 100% concentration or may be diluted for convenience using, for example, a distillate fuel. The diluent should be a clean-burning hydrocarbon, preferably a straight run petroleum distillate.

As indicated earlier, the present invention utilizes a 40 reaction product which is formed by reacting an inorganic salt of a type described hereinabove with a sulfonate of a type also described hereinabove. This reaction is preferably carried out by admixing proportions of an aqueous solution of one or more of the inorganic salts with an oil solution of one or more of the sulfonates and thereafter heating the resulting mixture at a temperature and for a period of time sufficient to vaporize all of the water from the mixture. Temperatures and reaction times that are suitable for this reaction depend to some extent upon the amount of water present in the reaction mixture, but reaction times of about 30 to 240 minutes and temperatures above 230° F. (preferably about 300° F.) are effective for the purpose.

55 The concentrates of the inorganic salts and the sulfonates within the respective aqueous and oil solutions have not been found to be critical to the success of the invention; but it is generally contemplated that substantially saturated solutions of the inorganic salts and oil solutions 60 containing about 25 to 100 wt. percent of the sulfonates are preferred. The solvents employed in the oil solutions of the sulfonates may include any conventional clean-burning petroleum distillate fraction and are conveniently petroleum fractions that boil in substantially the same 65 boiling range as the fuel oil components with which they are to be eventually blended.

The proportions of inorganic salts and sulfonates within the reaction involving these two compounds should be such as to provide about 0.1 to 4.0 mols of inorganic salt per mol of sulfonate and preferably about 0.5 to 2.5 mols of inorganic salt per mol of sulfonate.

The structure of the reaction product that is formed by admixing and heating the inorganic salt and the sulfonate in the manner described above is not presently known, 75 but it appears that a coordination complex of some sort

is formed which possesses the very desirable quality of being very soluble in distillate petroleum fractions of the type of interest here. It should be noted at this point that a portion of the inorganic salt may fail to go into solution during the reaction period, and this insoluble portion should be separated, as by filtering or centrifuging, from the reaction product before the latter material is incorporated within a distillate fuel.

The complex reaction product may be incorporated in a distillate fuel oil of a type described earlier herein by any suitable conventional procedure. Thus, propeller mixers, micronizers, conventional stirring devices, etc. and mild-heating may be employed for this purpose. It is important, however, that a sufficient portion of the reaction product be incorporated in the fuel oil so as to achieve the objectives of the invention. The exact amounts required for this purpose may vary slightly depending upon the nature of the fuel oil; but an amount in excess of about 0.002% by weight of active ingredient is generally required. Amounts of the reaction product up to about 0.3 wt. percent may be employed, but the advantages of the invention are best realized with amounts of about 0.01 to 0.10 wt. percent and especially about 0.02 wt. percent based on active ingredient.

While the foregoing description has been concerned with a preferred procedure wherein an aqueous solution of an inorganic salt is reacted with an oil solution of a sulfonate, it will be appreciated that variations from this procedure may be resorted to without departing from the spirit or scope of the invention. Thus, it is possible that the inorganic salt may be introduced directly within the sulfonic acid salt solution in dry form without utilizing an aqueous solution of the salt. Furthermore, in some instances, it may be desirable to employ an alcoholic solution of the salt rather than an aqueous solution. Again, it may be desirable to form the complex reaction product directly within the distillate fuel oil itself; and it may also be desirable to aid water removal from the reaction mixture by bubbling a dry gas such as nitrogen or the like through the reaction mixture during the heating period.

It will also be appreciated that a number of other conventional fuel oil additives such as drying agents, color stabilizers, demulsifying agents, oiliness agents, etc. may also be incorporated within the present compositions so long as these other materials do not interfere with the objectives of the invention.

In order to better illustrate the nature of the present invention, attention is directed to the following examples wherein samples of a distillate fuel oil were evaluated with particular reference to their sediment stability, color hold and corrosion inhibiting qualities. The samples of fuel oil in some instances contained no additives and in other instances contained additives of the prior art. In still other instances, samples of the fuel oil were provided with the complex reaction product additives of the type described in the present invention.

The distillate fuel oil that was employed in these examples had the following physical characteristics:

|                      |        |
|----------------------|--------|
| Gravity, °API        | 32     |
| Boiling pt., initial | °F 330 |
| 10% off @            | °F 413 |
| 50% off @            | °F 502 |
| 90% off @            | °F 594 |
| Final b. pt.         | °F 658 |
| Sulfur, wt. percent  | 0.8    |
| Flash pt.            | °F 150 |
| Color, Robinson      | 13     |
| Neut. No             | 0.03   |
| Vis. @ 100° F., SUS  | 32     |

The fuel oil was furthermore characterized by containing about 50 vol. percent straight run stocks, 40-45 vol. percent stocks from catalytic cracking operations and 5-10 vol. percent stocks from thermal cracking operations.

### EXAMPLE I

In a first series of tests, samples of the above fuel oil were evaluated alone and also in combination with several additives. For the sake of clarity, these additives are described separately in the following paragraphs and are designated by the letters A, B and C in order to further simplify the description. One of the additives employed in this example was the ammonium salt of an alkylated monocyclic aryl sulfonic acid of about 450 molecular weight. This additive consisted principally of ammonium didodecyl benzene sulfonate in about 40 wt. percent concentration in a straight run kerosene fraction. The additive is hereinafter referred to as additive A.

The second additive employed in the example was a complex reaction product formed by reacting 20 parts by weight of sodium nitrite (dissolved in 30 parts by weight of water) with 100 parts by weight of the above ammonium sulfonate (in 40 wt. percent concentration in a kerosene of 39° API and 325°-550° F. boiling range). In the preparation of this additive, which constitutes an additive of the present invention, the mixture of aqueous nitrite and sulfonate was heated to a temperature of 300° F. with continuous stirring and with a light nitrogen blowing operation for a period of about one hour in order to remove water from the reaction mixture. Following the reaction period, the mixture was filtered to remove unreacted sodium nitrite. The resulting product was clear and contained about 5.7% by weight sodium and about 4.0% by weight sulfur. The calculated composition of this product, based on the analysis and the approximate molecular weight of 450 for the original ammonium sulfonate, is about 74% active ingredient of the reaction product of ammonium sulfonate and sodium nitrite and about 26% of the kerosene diluent. It will be noted that a portion of the kerosene is normally lost during the water removal operation, but this loss does not adversely affect the formation of the desired reaction product in any way. It will further be noted that this additive is hereinafter designated as additive B.

The third additive employed in this example was a prior art additive containing sodium petroleum sulfonate in combination with an alkyl phenol sulfide. The sodium sulfonate in this instance was the sodium salt of a petroleum sulfonic acid of about 500 molecular weight, and the phenol sulfide was present in the form of the salt of an alkaline earth metal. The additive furthermore consisted of about one part by weight of the sulfonate per two parts by weight of the phenol sulfide. This additive is hereinafter referred to as additive C.

In this example as will be described in detail, the various fuel oil compositions were evaluated in accordance with several methods—both as to their sediment stability and color hold and also as to their ability to inhibit the corrosion of ferrous metals.

In a first procedure, samples of the fuel compositions were heated for a period of about 16 hours at 210° F. and the sediment formed during the storage period thereafter recovered and weighed. It has been determined by an extensive number of samples that results from this test procedure correlate with actual sedimentation results that occur in fuel oils of this type during extended storage periods in actual storage tanks, domestic heating oil tanks, etc.

The corrosion inhibiting qualities of the various fuel samples were determined in accordance with a laboratory test procedure which has also been found to correlate with the actual field results that have been experienced by refiners and consumers of these products. In accordance with this procedure, a sample of fuel is vigorously admixed with about 5 vol. percent water (either distilled or synthetic sea water prepared as per ASTM-D-665-52T), and the resulting mixture is thereafter separated into an equilibrated oil layer and an equilibrated water layer. Each of the layers is reserved for subsequent use in the test.

For each fuel sample, a hot-rolled steel panel having its surface uniformly covered with an oxidized film or "mill scale" is used. Small spaced portions of the surface of the steel panel or test sample are descaled as by scratching or milling through the scale layer. A droplet of equilibrated water from the mixing operation described above is then placed directly on a part of each area of exposed fresh metal surface in such a way that the droplet also covers a part of the area of metal still covered with the deposited film.

Each steel panel or sample with its adhering droplets of water is then stored for a period of 21 days submerged beneath the surface of the equilibrated oil. Each point where a droplet is in contact with the bared metal plate is considered as a possible site of corrosion, and a total of about 1 to 16 corrosion sites is generally observed on each plate.

This arrangement of oil and water, each contacting a portion of each of the areas of exposed or film-covered metal, particularly favors the development of pitting corrosion which probably occurs through a mechanism involving electrical concentration cells. Pitting of actual metal surfaces in storage tanks is considered to proceed by this type of mechanism.

Following the storage time, each steel panel is removed from the oil and washed with pentane and acetone solvent. Each washed plate is then wire brushed to remove rust from the corrosion sites and is thereafter dried and weighed to determine the amount of metal lost due to corrosion. The depth of maximum corrosive penetration at each corrosion site is determined by means of a microscope which is equipped with a focusing dial calibrated in milliinches.

An additional test that was performed on each oil composition was a color hold test carried out in accordance with the following procedure. A sample of about 20 cc. of an oil composition is placed in the sample tube of a suitable colorimeter (a suitable instrument is the Hellige Diller Photoelectric Colorimeter—Model No. 400). With the sample in the sample tube, the instrument is adjusted to transmit white light through the sample, and suitable adjustments are made to indicate 100% light transmission for the fresh oil sample as a standard. A previously prepared sample of heat-treated (210° F. for 16 hours) and filtered oil from the same composition is then introduced into a sample tube and the percent light transmission again read from the instrument. The color hold value is then the percent light transmission through the heated and filtered test sample relative to the fresh sample, considering the latter sample to possess 100% light transmission.

The results that were obtained by subjecting the afore-described fuel compositions—i. e. the fuel oil itself and in combination with additives A, B and C—are presented in the following table.

Table I

## STABILITY AND CORROSION CHARACTERISTICS OF FUEL OIL COMPOSITIONS

| Additive                                                   | Base Fuel | A     | B     | C     |
|------------------------------------------------------------|-----------|-------|-------|-------|
| Additive Concentration: Wt. percent Active Ingrd.          | 0         | 0.025 | 0.022 | 0.02  |
| Storage Test, 16 hrs. @ 210° F.: Sediment, mgs./600 g. oil | 41.7      | 155.5 | 1.7   | ----- |
| Color hold, 16 hrs. @ 210° F.: Percent Transmission        | 58        | 8     | 71    | ----- |
| Pitting in Distilled Water:                                |           |       |       |       |
| Av. Max. Penetrat'n, Mils.                                 | 3.5       | 0     | 0     | 4.8   |
| Range of Max. Penet., Mils.                                | 2-5       | 0     | 0     | 2-11  |
| Wt. loss per site, mgs.                                    | 7.3       | 17.7  | 0     | 1.5   |
| No. of possible corrosion sites                            | 20        | 2     | 32    | 14    |
| Pitting in Synthetic Sea Water:                            |           |       |       |       |
| Av. Max. Penetration, Mils.                                | 1.7       | 1     | 0     | 2.2   |
| Range of Max. Penet., Mils.                                | 2-5       | 1     | 0     | 2-3   |
| Wt. Loss per site, mgs.                                    | 6.4       | 1.4   | 0     | 5.1   |
| No. of possible corrosion sites                            | 20        | 2     | 32    | 22    |

(1) Weight loss without pitting is primarily due to uniform corrosion of exposed metal areas.

It is readily apparent from the above table that the complex reaction product additive of the present invention is extremely effective in stabilizing a distillate fuel oil insofar as its sedimentation and colorhold characteristics are concerned. It is further apparent that this complex additive is extremely effective in reducing the degree of pitting corrosion that has otherwise been observed to occur in the presence of ferrous metals.

It will further be observed that ammonium sulfonate alone, as represented by sample A, possesses reasonably satisfactory pitting corrosion characteristics; but this additive is substantially ineffective in reducing sediment formation and colorhold depreciation. It will be appreciated that this particular additive has been suggested in the prior art for use as a sediment stabilizing additive in distillate fuels, but in the particular fuel tested here and in the additive concentration employed, this additive actually was detrimental in its effect rather than beneficial.

Table 1 above further demonstrates that the additives of the present invention are superior to another prior art additive—namely, an additive mixture of sodium petroleum sulfonate and the metal salt of an alkyl phenol sulfide. The latter additive has previously been demonstrated to possess good sediment and colorhold stabilizing properties, but it is markedly inferior to the present additive composition in reducing pitting corrosion.

At this point it is well to note that the complex additives of the present invention are also superior to an inorganic salt alone such as sodium nitrate in that salts of this type are not soluble in distillate mineral oils. It is conceivable, of course, that layers of water within storage tanks and the like could be provided with inorganic corrosion inhibitors such as sodium nitrite, but this mode of corrosion prevention is patently inferior to the present method for a number of obvious reasons.

What is claimed is:

1. An improved fuel composition comprising a major proportion of distillate petroleum hydrocarbons and a minor but sediment-stabilizing and rust-inhibiting proportion of an oil-soluble complex formed by reacting a water-soluble salt of nitrous acid with an oil-soluble ammonium sulfonate, the cationic portion of said nitrite being selected from the class consisting of the ammonium radical, sodium, lithium and potassium, the sulfonate being selected from the class consisting of the ammonium salts of the alkyl mono- and bi-cyclic aryl sulfonic acids, said complex being formed by conducting said reaction at a temperature and for a period of time sufficient to remove all of the water from the reaction mixture.
2. A composition as defined in claim 1 in which the alkyl portion of the sulfonate contains up to about 40 carbon atoms.
3. A composition as defined in claim 1 in which the complex is formed by reacting about 0.1 to 4.0 mols of the nitrite per mole of sulfonate.
4. A composition as defined in claim 1 in which the reaction product constitutes from about 0.002 to 0.3 wt. % of said composition.
5. A composition as defined in claim 1 in which the nitrous acid salt is sodium nitrite and the sulfonate is ammonium didodecyl benzene sulfonate.
6. A composition as defined in claim 1 in which the nitrite is ammonium nitrite and the sulfonate is ammonium didodecyl benzene sulfonate.
7. A composition as defined in claim 2 in which the alkyl portion is derived from the polymerization of an olefin.
8. An improved fuel composition comprising a major proportion of distillate petroleum hydrocarbons including at least about 10% cracked stocks and a minor proportion of an oil-soluble complex, said complex being formed by reacting an aqueous solution of a water-soluble nitrite with an oil-soluble ammonium sulfonate,

the cationic portion of the nitrite salt being selected from the class consisting of the ammonium radical and the alkali metals, the sulfonate being selected from the class consisting of the ammonium salts of alkyl mono- and di-cyclic aryl sulfonic acids, the reaction product being present in an amount less than 0.3 wt. % of said fuel composition but sufficient to prevent sediment formation and to inhibit the corrosion of metals with which the composition comes in contact, the reaction product being formed by conducting said reaction at a temperature and for a period of time sufficient to remove all of the water from the reaction mixture.

9. A composition as defined in claim 8 in which the sulfonate is derived from a petroleum sulfonic acid of about 300 to 650 molecular weight. 15

## References Cited in the file of this patent

## UNITED STATES PATENTS

|              |                |                |
|--------------|----------------|----------------|
| 2,296,069    | Talbert et al. | Sept. 15, 1942 |
| 2,297,666    | Wachter        | Sept. 29, 1942 |
| 5 2,527,987  | Carom et al.   | Oct. 31, 1950  |
| 2,616,924    | Asseff et al.  | Nov. 4, 1952   |
| 2,623,016    | Mertes         | Dec. 23, 1952  |
| 2,650,198    | Kronig et al.  | Aug. 25, 1953  |
| 10 2,695,910 | Asseff et al.  | Nov. 30, 1954  |
| 2,742,351    | Rogers et al.  | Apr. 17, 1956  |

## FOREIGN PATENTS

|           |        |               |
|-----------|--------|---------------|
| 1,055,483 | France | Feb. 18, 1954 |
|-----------|--------|---------------|